

# UNITED STATES PATENT OFFICE.

ISAAC M. SCOTT, OF WHEELING, WEST VIRGINIA.

## METHOD OF SIMULTANEOUSLY ANNEALING AND DESCALING TIN-PLATE.

1,359,282.

Specification of Letters Patent. Patented Nov. 16, 1920.

No Drawing.

Application filed June 30, 1920. Serial No. 392,987.

To all whom it may concern:

Be it known that I, ISAAC M. SCOTT, a citizen of the United States, residing at Wheeling, in the county of Ohio and State of West Virginia, have invented certain new and useful Improvements in Methods of Simultaneously Annealing and Descaling Tin-Plate; and I do hereby declare the following to be a full, clear, and exact description 10 of the invention, such as will enable others skilled in the art to which it appertains to make and use the same.

This invention relates to a method of annealing and simultaneously removing oxids 15 of iron from the surface of iron and steel plates and has for its object to improve the processes heretofore proposed.

With this and other objects in view the invention consists in the novel steps and 20 combinations of steps constituting the process, all as will be more fully hereinafter disclosed and particularly pointed out in the claims.

In order that the precise invention may be 25 the more clearly understood it is said: It is well known that thin iron or steel plates, commonly known as tin plates, have to be subjected to separate annealing and descaling processes before they are ready for the 30 tin bath, and that these separate treatments constitute an important item in the cost of their manufacture. It is the object of this invention, when more particularly stated to reduce this said item of cost by performing 35 the annealing and descaling operations simultaneously. In order to accomplish this, I may lay the plates flat in the annealing boxes and sprinkle by a suitable means, finely divided carbon successively on their 40 surfaces, so that the pile when built up will consist of alternate layers of plates and films of carbon dust; or I may lay the plates flat in the boxes without any carbon between them, and then turn the boxes and plates 45 on edge and sprinkle carbon dust between. This latter operation is facilitated by the unevennesses between the surfaces of the plates produced by the rolling process. As a further alternative method, I may make 50 a thin paste of finely divided carbon and water, and wash or coat the plates therewith in any suitable manner, as by dipping, flowing the paste over the plates, or otherwise applying it to them, after which the plates 55 are placed in the annealing boxes and passed on into the annealing oven, where they are

heated to a sufficient temperature to cause the carbon to react with the iron oxids, substantially in accordance with the following equations:—



The temperature required must be not less than say 450° C. to effect a velocity of reaction capable of industrial application, but the temperature may rise to 1000° C. or even somewhat higher, so long as the softening temperature of the iron or steel is not reached.

After the annealing operation is completed, the plates will be found free from scale and coated in its place with very thin films of iron, which will serve as protectors for the plates against further oxidations. 70 The carbon remaining between the plates is readily removed during the subsequent cleaning operations, and some of it is found to enter the surfaces of the plates, but not to an objectional extent. After the plates have 80 been thus annealed and descaled, they are put through the other well known process preparatory to the coating with tin in the customary ways.

My invention also includes the annealing 85 or other heat treatment of iron or steel simultaneously with the reduction of iron oxids, by varying the period of cooling, method of quenching, or other treatment during heating or cooling, to realize an in- 90 dustrially useful effect.

In such cases I prefer to embed the shaped metal in pulverized dry coke, charcoal, or other forms of commercial carbon, or carbonaceous matter; but I may also dip such 95 metal shapes in a finely divided carbon or carbonaceous material suspended in water, oil, or other liquid vehicle, in order to cover such shapes when in forms to permit such a procedure. Such shapes, when in the forms 100 of sheets, plates, etc., may be passed through rolls, or other coating applying means, which are constantly supplied with a carbonaceous matter in the form of a thick paste or emulsion. In such cases the treatment is some- 105 what analogous to the inking of type faces in the process of printing.

My process of simultaneously annealing and descaling metal forms may be operated in an ordinary annealing, or other type of 110 direct heat furnace, or in a muffle furnace, or in a sealed furnace heated from without,

or by electric means within the furnace chamber. Said process may also be carried out in an atmosphere of ordinary fuel combustion products, or in a vacuum, or in an atmosphere composed of inert gases, such as nitrogen, hydrogen, carbon monoxid, natural gas, etc., or in other gases which cannot cause oxidation of the metal. Said process, also may be readily carried out under conditions capable of controlling or regulating the mixture and concentration of such gases.

10 My process is likewise carried out at such temperatures and under such times of treatment as will preclude any serious carburization of the metal shapes, unless such carburization is desired.

15 What I claim is:—

1. The process of simultaneously annealing and descaling tin plate which consists in packing said plate in annealing boxes with carbonaceous material between them; and then subjecting said plates to annealing temperatures sufficient to reduce the scale pres-

ent, but insufficient to carbonize the plate to a substantial extent, substantially as de- 25 scribed.

2. The process of simultaneously annealing and descaling tin plate, which consists in placing said plate into annealing boxes; placing finely divided carbon between the individual plates; and passing the packs of plates thus formed through the usual annealing process, substantially as described.

3. The process of simultaneously annealing and descaling iron and steel forms which consists in coating the surfaces of said forms with a wet carbonaceous material, and then subjecting the coated forms in an atmosphere of reducing gas to the action of annealing temperatures sufficient to reduce the scale present but insufficient to materially carburize said forms, substantially as described.

35 In testimony whereof I affix my signature.

ISAAC M. SCOTT.